

# UNITED STATES PATENT OFFICE.

OMA CARR, OF ASHEVILLE, NORTH CAROLINA.

## MANUFACTURE OF SULFITE PULP FROM RESINOUS WOODS.

1,089,691.

Specification of Letters Patent. Patented Mar. 10, 1914.

No Drawing.

Application filed August 9, 1913. Serial No. 783,900.

*To all whom it may concern:*

Be it known that I, OMA CARR, a citizen of the United States of America, residing at Asheville, county of Buncombe, State 5 of North Carolina, have invented certain new and useful Improvements in the Manufacture of Sulfite Pulp from Resinous Woods, of which the following specification is a clear description.

10 Practically all resin-bearing woods store the greater part of their resin in the "summer" ring of the wood, the rest being stored in the medullary rays. Wherever the resins are stored the cellulose is stained yellow or 15 yellow-brown. In many varieties of pine this stain is of such character that it does not dissolve out under the action of the sulfite "cook liquor," the stained fibers being only partially cooked and eventually 20 showing in the pulp as "shieves" or "yellow shiners." These pines are not, therefore, available for pulp by the sulfite process in their natural state; and as they are very 25 abundant, of rapid growth, and of insignificant value for lumber or fuel use, it is economically desirable to render them suitable.

It is the object of my invention to attack the "yellow ring," or stained fibers, before 30 subjecting the wood to the sulfite cook, the desirable characteristics of which, as compared with the soda process, are well known. This I accomplish by the use of turpentine and alkali in combination. The resins causing the stain are complex in chemical 35 composition, some being acid in nature and soluble in alkaline solvent, while others act as neutral resins and are soluble in turpentine.

An outline of one general method of procedure is as follows: The wood is chipped in the usual way and the chips placed in an autoclave (one of a series); they are then extracted by turpentine, a large part of the resins responding to this solvent, heat and circulation promoting the result. Following the turpentine extraction I place on the chips a solution of alkali (common soda ash 45 is convenient, but caustic soda is more effective), and by heat and circulation remove the remaining resins. The extraction may be conducted with the autoclaves as a series, inter-connected, or intermittently, the alkali solvent may precede the turpentine, or, the

two solvents may be used together, the turpentine emulsifying with the alkali solvent. 55

A specific procedure may be as follows: A battery, or series, of autoclaves is employed, preferably eight in number and interconnected by appropriate piping and provided with heaters and valves. Numbers one to six 60 will contain chips submerged in alkaline solvent, numbers seven and eight chips submerged in turpentine solvent. By means of compressed air the solvent in number one is forced forward, a "draw" of alkaline solvent being taken from number six; simultaneously fresh turpentine solvent is forced into number seven and a "draw" of such solvent taken from number eight. Then number one is "dumped" of its charge of 70 "spent" chips, and filled with fresh, or unextracted, chips. Number eight is now connected with number one, and by running fresh alkaline solvent into number two circulation is forced through the battery and tur- 75 pentine solvent from number eight is forced over into number one, saturating the fresh chips there. The battery is now ready for compressed air in number two, a "draw" of alkaline solvent from number seven; fresh 80 turpentine solvent into number eight, and a "draw" of turpentine solvent from number one. Thus the extraction proceeds, the fresh chips being bathed in turpentine solvent and the nearly spent chips bathed in 85 alkaline solvent. The "draw" of alkaline solvent contains resins as soaps, and residual turpentine; the turpentine is recovered by appropriate distillation, and by evaporation the resin soaps are obtained. The "draw" 90 of turpentine solvent contains resins, and by distillation of the turpentine the resins are obtained in the "free" state. Whatever turpentine is contained in the wood primarily, is collected and appears in the turpen- 95 tine reclaimed.

The "spent" chips are practically free of resin and yellow stain, and after draining or drying may be cooked by the conventional sulfite process.

Obviously the process may be reversed, the alkaline solvent preceding the turpentine solvent, while it is also apparent that the two solvents may be merged together; and it is further apparent that the extraction 105 may be conducted in an intermittent man-

ner instead of serially. The specific procedure described above, however, gives best results.

Having described my invention, what I claim as new and desire to secure by Letters Patent is:

The method herein described of making sulfite pulp from resinous woods, consisting in dissolving out the resinous matters by

subjecting the wood chips to turpentine and 10 also an alkaline solvent, and then cooking the chips by the sulfite process.

In testimony whereof I hereunto affix my signature in the presence of two witnesses.

OMA CARR.

Witnesses:

JOHN T. SMITH, Jr.,  
R. M. ROBERTS.